

## UNITED STATES PATENT OFFICE

GEORGE LUTZ, OF ROCKY RIVER, AND LEON R. WESTBROOK, OF CLEVELAND HEIGHTS, OHIO, ASSIGNORS, BY MESNE ASSIGNMENTS, TO THE GRASSELLI CHEMICAL COMPANY, OF CLEVELAND, OHIO, A CORPORATION OF DELAWARE

## ELECTROPLATING

No Drawing.

Application filed February 23, 1928. Serial No. 256,476.

This invention relates to addition agents useful in the commercial production of electroplates on metals.

It is customary to add certain organic more or less colloidal addition agents to electroplating baths. The function of these agents is not well understood, and no general rule is known which would give a lead as to the type of compounds to be used or the conditions under which the most beneficial results can be obtained. The addition of such agents to plating baths results, however, in electroplates of very desirable properties which could not be duplicated without them, and hard, mirror-like perfectly adherent deposits are, in many instances, only due to the use of such addition agents. Such agents do not act the same in every type of bath or produce like results with all metals. It is usually necessary to adjust the composition of the bath for every particular addition agent, and to duplicate or obtain uniform results strict adherence to the predetermined conditions is essential.

We have now found that certain alkylated naphthalene sulfonic acids and their water soluble salts are well suited for use as addition agents in electroplating processes.

Alkyl naphthalene sulfonic acids in which the alkyl group contains more than two carbon atoms are easily prepared and are commercially available in the form of their sodium salts. Propyl, butyl, cyclohexyl, and benzyl naphthalene sulfonic acids are typical representatives of this group of compounds.

Our invention consists now in the addition of relatively small amounts of such alkylated naphthalene sulfonic acids to electroplating baths and in the novel baths so obtained.

Electroplates obtained from such baths show usually an improved hardness, brightness, and better adherence of the plate on the base metal.

The alkyl naphthalene sulfonic acids or their salts are soluble only to a limited extent in certain electroplating baths, in which instances the more soluble compounds, such as the benzyl-naphthalene sulfonic acids, are preferred as the amounts of the less soluble compounds which would go in solution might

be insufficient to produce the full beneficial effect obtained in our baths.

Valuable results have been obtained in alkaline cyanide baths as well as in acid baths. There again the composition of the bath as well as the particular alkyl naphthalene sulfonic acid used will have to be adjusted, and this can be done by a few experiments.

The following examples will further illustrate our invention by showing the application of the alkyl naphthalene sulfonic acids to various electroplating processes. It is understood that our invention is not limited to these particular baths, but that similar beneficial results can be obtained in other electroplating solutions by the addition of alkyl naphthalene sulfonic acids thereto.

(1) A cadmium cyanide bath was prepared containing

|                                      |     |                  |    |
|--------------------------------------|-----|------------------|----|
| NaCN                                 | 120 | grams            | 70 |
| Cd(OH) <sub>2</sub>                  | 48  | grams            |    |
| Na <sub>2</sub> SO <sub>4</sub>      | 60  | grams            |    |
| NiSO <sub>4</sub> ·7H <sub>2</sub> O | 1.5 | grams per liter; |    |

To this was added 1 gram of benzyl-naphthalene sodium sulfonate. This was electrolyzed with a current density of 15-30 amp. per sq. ft. at room temperature. A bright, hard, mirror-like plate was obtained on the steel cathode.

The relative amounts of nickel and addition agent are critical. 0.05% of the addition agent to 0.005 to 0.03% of nickel in the bath gives the desired plate.

By doubling the amount of the naphthalene compound the amount of nickel has to be increased to 0.02 to 0.05% to obtain a similar result.

(2) 1 gram of benzyl-naphthalene sodium sulfonate was added to each liter of a nickel plating bath containing

|                                      |     |       |
|--------------------------------------|-----|-------|
| NiSO <sub>4</sub> ·7H <sub>2</sub> O | 240 | grams |
| NiCl <sub>2</sub> ·6H <sub>2</sub> O | 15  | grams |
| H <sub>3</sub> BO <sub>3</sub>       | 30  | grams |

The pH of this bath was adjusted to 5.8 and it was electrolyzed with a current density of 5-20 amps. per sq. ft. at room temperature. The plates obtained from this bath on steel were brighter, smoother, more uniform, and

apparently harder than those obtained from the same bath in which the addition agent had been omitted.

5 The amount of benzyl-naphthalene sulfonic acid contained in this bath could be increased to about twice that used above without changing the result.

(3) Steel plates were electrolyzed in an acid zinc bath containing

10  $ZnSO_4 \cdot 7H_2O$  ----- 360 grams  
 $NH_4Cl$  ----- 30 grams  
 $NaC_2H_3O_2 \cdot 3H_2O$  ----- 15 grams  
 $H_2SO_4$  ----- 3 grams

15 Benzyl - naphthalene sodium sulfonate--- 1-5 grams per liter.

The bath was kept at room temperature and a current density of 15-30 amps. per sq. ft. used. Whiter, brighter and denser plates

20 were obtained than without the use of the addition agent.

(4) Propyl-naphthalene sodium sulfonate was added in amounts varying from 1 to 2 grams per liter to a nickel plating bath 25 containing

$NiSO_4 \cdot 7H_2O$  ----- 240 grams.  
 $NiCl_2 \cdot 6H_2O$  ----- 15 grams.  
 $H_3BO_3$  ----- 30 grams per liter.

30 The pH of this bath was adjusted to 5.8 and it was electrolyzed at a current density of from 5-20 amps. per sq. ft. at room temperature.

35 The addition of the naphthalene sulfonic acid to this bath had a decided beneficial effect in that the plates obtained on steel were brighter, smoother, more uniform, and harder than plates obtained without the use of the addition agent. They were quite similar to those obtained with the benzyl-naphthalene sulfonic acid.

(5) The addition agent used in Example 3 was replaced in the same bath by propyl-naphthalene sodium sulfonate in amounts 45 from 1 to 5 grams per liter, maintaining other conditions alike. The plates on steel were decidedly brighter and whiter than those obtained from the same baths in which 50 the addition agent had been omitted.

It is immaterial, for purposes of this invention, whether the free alkyl-naphthalene sulfonic acids or their water soluble salts are used as addition agents to electroplating 55 baths; the actual compound contained in the bath will depend upon the alkalinity or acidity of the bath, and the term alkyl naphthalene sulfonic acid as used herein is meant to embrace the free acids as well as their water 60 soluble salts or derivatives. It is furthermore understood that the term alkyl, as used herein, includes ar-alkyl radicals such as benzyl and other saturated hydrocarbon radicals.

65 We claim:

1. An alkyl-naphthalene sulfonic acid as an addition agent to an electroplating bath.

2. An alkyl-naphthalene sulfonic acid, in which the alkyl group contains more than two carbon atoms, as an addition agent to an 70 electroplating bath.

3. An electroplating bath comprising an aqueous solution of a compound of a metal to be deposited by electrolysis, said solution containing an alkyl-naphthalene sulfonic 75 acid.

4. An electroplating bath comprising an aqueous solution of a compound of a metal to be deposited by electrolysis, said solution containing an alkyl-naphthalene sulfonic 80 acid in which the alkyl group contains more than two carbon atoms.

5. The process of electroplating which comprises electrodepositing a metal from an aqueous solution of a compound of a metal 85 to be deposited, said solution containing an alkyl-naphthalene sulfonic acid.

6. The process of electroplating which comprises electrodepositing a metal from an aqueous solution of a compound of a metal 90 to be deposited, said solution containing an alkyl-naphthalene sulfonic acid in which the alkyl group contains more than two carbon atoms.

7. An aqueous cadmium cyanide electroplating bath containing in solution an alkyl naphthalene sulfonic acid compound in which the alkyl group contains more than 95 two carbon atoms.

8. An aqueous nickel electroplating bath 100 containing in solution an alkyl naphthalene sulfonic acid compound in which the alkyl group contains more than two carbon atoms.

9. An aqueous acid zinc electroplating bath containing in solution an alkyl naphthalene sulfonic acid in which the alkyl group contains more than two carbon atoms. 105

In testimony whereof, we affix our signatures.

GEORGE LUTZ.  
 LEON R. WESTBROOK.

110

115

120

125

130